

1

3,419,390

## ELEMENTS AND DEVELOPERS FOR COLOR PHOTOGRAPHY UTILIZING PHENOLIC COUPLERS CONTAINING AN AMINOALKYL GROUP ON THE COUPLING POSITION

Homer W. J. Cressman and John R. Thirtle, Rochester, N.Y., assignors to Eastman Kodak Company, Rochester, N.Y., a corporation of New Jersey

No Drawing. Continuation-in-part of application Ser. No. 452,932, May 3, 1965. This application Oct. 4, 1965, Ser. No. 492,904

13 Claims. (Cl. 96—55)

## ABSTRACT OF THE DISCLOSURE

Cyan dye-forming phenolic and naphtholic couplers having an aminomethyl substituent attached to the active carbon of the couplers are used to advantage in color photography to form nondiffusible cyan dye images in color photographic elements because of their high coupling reactivity and very low density of unwanted color fog that is formed by color development.

This is a continuation-in-part application of Homer W. J. Cressman and John R. Thirtle, U.S. Ser. 452,932, filed May 3, 1965, now abandoned.

This invention relates to color photography and more particularly to new and improved cyan dye-forming coupler compounds for the formation of images.

The formation of colored photographic images by the imagewise coupling of oxidized aromatic primary amino developing agents with color-forming or coupling compounds to form indophenol, indoaniline, and azomethine dyes is well known. In these processes, the subtractive process of color formation is ordinarily used and the image dyes customarily formed are cyan, magenta, and yellow, the colors that are complementary to the primary colors, red, green, and blue, respectively. Usually phenol or naphthol couplers are used to form the cyan dye image; pyrazolone or cyanoacetyl derivative couplers are used to form the magenta dye image; and acylacetamide couplers are used to form the yellow dye image.

In these color photographic systems, the color-forming coupler may be either in the developer solution or incorporated in the light-sensitive photographic emulsion layer so that, during development, it is available in the emulsion layer to react with the color developing agent that is oxidized by silver image development. Diffusible couplers are used in color developer solutions. Nondiffusing couplers are incorporated in photographic emulsion layers.

It is an object of our invention to provide new and improved couplers capable of forming cyan dye with the oxidation product of a primary aromatic amino color developing agent.

It is a further object to provide new and improved low-fogging cyan couplers with good reactivity so that processing can be accomplished in a reasonable time and without prolonging development or without requirement for excessively high pH or high temperature processing conditions.

Another object is to provide new aminoalkyl substituted four-equivalent couplers which have good coupling reactivity and which include the diffusible type coupler, the Fischer-type and the nondiffusing type couplers which are readily incorporated in light-sensitive hydrophilic colloid-silver halide emulsion layers by means of a wide range of coupler-to-solvent ratios.

Still another object of our invention is to provide new uncolored cyan-dye-forming couplers which afford automatic color correction for the cyan dye image.

2

Another object is to provide new image-forming layers containing our new couplers alone or in a hydrophilic colloid such that the coupler is contiguous to light-sensitive silver halide, ZnO, ZnS, CdS, CdSe, NiS, etc., either with or without a binder.

Still another object is to provide improved cyan dye photographic images and improved multicolor photographic images by the use of these new couplers.

Another object is to provide new diffusible cyan image-forming couplers for use in cyan color developer solutions.

Still further objects will be apparent from the following specification and claims.

These and other objects are accomplished according to our invention by the use of our new class of four-equivalent phenolic cyan-dye-forming coupling agents in photographic dye-image-forming systems. The compounds of our invention have good coupling reactivity and a low incidence of color fog. Our couplers are characterized by having at least one phenolic coupling moiety with an aminoalkyl group on the coupling position(s) which is displaced when the coupler reacts with oxidized color developer.

The fact that phenolic compounds containing an aminoalkyl group in the coupling position couple with oxidized color developing agents to form cyan dye is unexpected since it had previously been understood that alkyl groups in the coupling position are not displaceable and dye formation does not take place.

Our new cyan-dye-forming couplers are derived from any of the known phenolic or naphtholic cyan-forming four-equivalent couplers by substituting an aminoalkyl group on the carbon atom in the coupling position of the coupler, the said amino group having at least one hydrogen atom.

Included among the new and improved cyan-dye-forming couplers of our invention are those shown to advantages by the formulas:

I.



II.



The R group in the above formula represents an alkoxy group, either straight or branched chain, particularly those of from 1 to 22 carbon atoms (e.g., ethoxy, isopropoxy, decyloxy, octadecyloxy, docosoxy, etc.), a mono or bicyclic alkoxy group such as cyclohexyloxy, cyclopentoxy, norbornyloxy, etc. The alkoxy group may contain substituent groups such as halogen, nitro, hydroxyl, carboxyl, amino, carboxyl ester, e.g., carbomethoxy, sulfo, sulfo esters, e.g., methoxysulfonyl, alkoxy as hereinabove defined, amide, etc. such that when the R group is a carboxyl or sulfo substituted alkoxy group, the coupler contains sufficient ballasting to render a dye from said coupler nondiffusing. The R group may also represent an amide group such as acetamido, ethylsulfonamido, N-methylbutyramido, N-propylbenzamido, 4-t-butylbenzamido, carbamyl, N-octadecylcarbamyl, N,N-dihexylcarbamyl, N-

methyl-N-phenylcarbamyl, 3-pentadecylphenylcarbamyl, sulfamyl, etc., such that when R represents sulfamyl, the coupler contains sufficient ballasting to render a dye from said coupler nondiffusing. These amide groups may also be substituted with groups such as defined for the substituted alkoxy group in R above (e.g., halogen, nitro, hydroxyl, carboxyl, amino, carboxyl esters, sulfo esters, amide, etc.). The R' group represents a hydrogen atom, an alkyl group, either straight or branched chain of from 1 to 22 carbon atoms (e.g., methyl, ethyl, isopropyl, tertiary butyl, dodecyl, docosyl, etc.), a mono or bicyclic alkyl group such as cyclopentyl, norbornyl, etc., or an aryl group such as phenyl, napthyl, etc. These groups, i.e., alkyl and aryl, may also be substituted with groups such as defined for the substituted alkoxy groups in R above. The R<sup>2</sup> and R<sup>3</sup> groups each represent the hydrogen atom, a halogen atom, an alkyl, aryl, alkoxy, or amide group as defined in R and R' above. The R<sup>2</sup> and R<sup>3</sup> groups may also represent the non-metallic atoms needed to complete a fused ring, such as a 5,6- and 6,6-membered isocyclic and heterocyclic rings, e.g., naphthalene, quinoline, benzothiazole, benzimidazole, etc.

Our phenolic (i.e., phenols and naphthols) couplers are characterized by having an amino alkyl group on the coupling position of the coupler which gives them good coupling reactivity and other valuable properties. These couplers are particularly characterized by the low levels of unwanted color fog produced. Excellent coupling reactivity is obtained with couplers of our invention when incorporated in emulsion layers without the use of high-boiling coupler solvents. When high-boiling solvents are used to disperse these couplers, high dye yield and low color fog are attained over a wide range of coupler-to-solvent ratios. When the diffusible couplers of our invention are used in color developing solutions, excellent reactivity and good dye yield are achieved.

Included among the couplers of Formulas I and II are the following typical examples used to illustrate but not limit our invention.

- (1) 4-aminomethyl-2-methoxyphenol
- (2) 4-butylaminomethyl-2-methoxyphenol
- (3) 4-anilinomethyl-2-methoxyphenol
- (4) 1-hydroxy-4-ethylaminomethyl-2-naphthamide
- (5) 2-ethoxy-4-propylaminomethyl-5-acetamido-1-naphthol
- (6)  $\alpha, \alpha'$ -iminobis (4-methyl-2-methoxyphenol)
- (7) 1-hydroxy-4-[N-(4-methoxyphenyl)aminomethyl]-N-[ $\delta$ -(2,4-di-t-amylphenoxy)butyl]-2-naphthamide



- (8) 1-hydroxy-4-[N-(4-methoxyphenyl)aminomethyl]-N-octadecyl-N-(3',5'-dicarbomethoxy)-2-naphthanilide
- (9) 1-hydroxy-4-[N-(3-methylphenyl)aminomethyl]-octadecyl-3',5'-dicarboxy-2-naphthanilide
- (10) 1-hydroxy-4-(N-methylaminomethyl)-2'-tetradecyloxy-2-naphthanilide
- (11) 1-hydroxy-4-[N-(tolyl)aminomethyl]-N-[ $\beta$ -{4-[2-(2,4-di-t-amylphenoxy)-5-(3-sulfonylbenzamido)-benzamido]-phenyl}ethyl]-2-naphthamide sodium
- (12) 2-benzamido-4-[N-(4-butylphenyl)aminomethyl]-5-[ $\alpha$ -(2,4-di-t-amylphenoxy)butyramido]phenol
- (13) 2-hexanamide-4-[N-(4-octadecyloxyphenyl)aminomethyl]-5-tetradecylsulfonamidopheno!

- (14) 2-[ $\gamma$ -(3-pentadecylphenoxy)butyramido]-4-[N-( $\delta$ -methoxybutyl)aminomethyl]-5-methylphenol
- (15)  $\alpha, \alpha'$ -iminobis{4-methyl-2-[ $\gamma$ -(4-t-butylphenoxy)butyramido]phenol}



- (16) 2-stearamido-4-[N-propylaminomethyl]-6-phenylphenol
- (17) 2-octadecyloxy-4-[N-(4-methoxyphenyl)aminomethyl]-1-naphthol
- (18) 5-(N-ethylaminomethyl)-7-acetamido-8-hydroxy-quinoline
- (19) 4-hydroxy-5-(N-butylcarbamyl)-7-(N-octadecylaminomethyl)benzimidazole



- (20) 1-hydroxy-4-[N-[4-(8-acetamido-3,6-disulfo-1-hydroxy-2-naphthylazo)phenyl]aminomethyl]-N-[ $\gamma$ -(2,4-di-t-amylphenoxy)butyl]-2-naphthamide disodium salt
- (21) 1-hydroxy-4-[N-(4-octadecyloxyphenyl)aminomethyl]-N-[B-(dimethylsulfamyl)ethyl]-2-naphthamide
- (22) 1-hydroxy-4-[N-(3-stearamidophenyl)aminomethyl]-2'-methoxy-2-naphthanilide
- (23) 1-hydroxy-4-(N-norbornylaminomethyl)-N-[ $\gamma$ -(3-pentadecylphenoxy)butyl]-2-naphthamide

The couplers of our invention are distinguished by their high reactivity and the very low density of unwanted color fog that is formed by color development to form dye images from the couplers. The aminoalkyl group provides a means of attaching other substituents to our couplers such as, for example, preformed dyes useful in color correction, and the like. Additional ballasting groups can conveniently be introduced via the aminoalkyl group; these ballasting groups are then eliminated during the coupling reaction with oxidized color developer which forms the image dyes.

The diffusible couplers of our invention, such as couplers 1-6, and 18, are used to advantage in color developer solutions used to color develop light-sensitive elements used for color photography which do not contain the color-forming coupler. Any of the well known primary aromatic amino color-forming silver halide developing agents such as the phenylenediamines, e.g., diethyl-p-phenylenediamine hydrochloride, monomethyl-p-phenylenediamine hydrochloride, dimethyl-p-phenylenediamine hydrochloride, 2-amino-5-diethylaminotoluene hydrochloride, 2-amino-5-(N-ethyl-N-lauryl)aminotoluene, N-ethyl- $\beta$ -methanesulfonamidoethyl - 3 - methyl - 4 - amino-

aniline, 4-N-ethyl-N- $\beta$ -hydroxyethylaminoaniline, etc., the p-aminophenols and their substitution products where the amino group is unsubstituted may be used in the alkaline developer solution with our couplers. Various other materials may be included in the developer solutions depending upon the particular requirements, for example, an alkali metal sulfite, carbonate, bisulfite, bromide, iodide, etc., and the thickening agents used in viscous developer compositions. The following is a typical developer solution given to illustrate but not limit our invention.

|                                   |      |
|-----------------------------------|------|
| 2-amino-4-diethylaminotoluene HCl | 2.0  |
| Sodium sulfite (anhydrous)        | 2.0  |
| Sodium carbonate monohydrate      | 20.0 |
| Potassium bromide                 | 1.0  |
| Coupler                           | 2.0  |
| Water to 1000.0 ml.               |      |

The other coupler examples used to illustrate our invention are nondiffusing and are used to advantage in photographic image-forming layers. Couplers such as 9, 11, 20 illustrate those that are incorporated as Fischer-type couplers. The other nondiffusing couplers, e.g., 7, 8, 10, 12, 13, 14, 15, 16, 17, 19, 21, 22, 23, are incorporated in emulsion layers by methods such as are described by Mannes et al., U.S. Patent 2,304,939, issued Dec. 15, 1942, Jelley et al., U.S. Patent 2,322,027, issued June 15, 1943, etc., in which high-boiling organic solvents are used to dissolve the coupler, and by methods described in Vittum et al., U.S. Patent 2,801,170, and Fierke et al., U.S. Patent 2,801,171, both issued July 30, 1957, and Julian, U.S. Patent 2,949,360, issued Aug. 16, 1960, in which low-boiling or water-soluble organic solvents are used with or in place of the high-boiling solvent. The use of such coupler dispersions permits thinner emulsion layers. These thinner layers are very desirable because they cause less light scattering, consequently, they produce sharper images.

Coupler 20 contains a preformed dye attached to the coupler on the phenylaminoalkyl group. This dye is eliminated on the coupling of the coupler with an oxidized color developer and diffuses out of the film. This coupler can be used as a magenta-colored coupler for the purpose of correcting for the unwanted green absorption of cyan image dyes, i.e., that formed from the coupler itself as well as that formed from other cyan couplers. Generally, such a coupler as this would be used in combination with another image-forming cyan coupler in the same layer.

Our couplers are used to advantage in the color development of photographic image-forming layers of the developing-out types. The light-sensitive materials used to advantage in our image-forming layers include silver halide (e.g., silver chloride, silver bromide, silver iodide, silver chlorobromide, silver bromoiodide, silver chlorobromoiodide, etc.), ZnO, ZnS, CdS, CdSe, NiS, etc., either with or without a hydrophilic colloid binder. When incorporated in image-forming layers, our couplers are contiguous with the said light-sensitive material either in the same layer or in a contiguous layer.

Hydrophilic colloids used to advantage include gelatin, colloidal albumin, a cellulose derivative, or a synthetic resin, for instance, a polyvinyl compound. Some colloids which may be used are polyvinyl alcohol or a hydrolyzed polyvinyl acetate as described in U.S. Patent 2,286,215, a far-hydrolyzed cellulose ester, such as cellulose acetate hydrolyzed to an acetyl content of 19-26%, as described in U.S. Patent 2,327,808, a water-soluble ethanolamine cellulose acetate as described in U.S. Patent 2,322,085; a polyacrylamide having a combined acrylamide content of 30-60% and a specific viscosity of 0.25-1.5 or an imidized polyacrylamide of like acrylamide content and viscosity as described in U.S. Patent 2,541,474, zein as described in U.S. Patent 2,563,791, a vinyl alcohol polymer containing urethane carboxylic acid groups of the

type described in U.S. Patent 2,768,154, or containing cyano-acetyl groups, such as the vinyl alcohol-vinyl cyanoacetate copolymer as described in U.S. Patent 2,808,331, or a polymeric material which results from polymerizing a protein or a saturated acrylated protein with a monomer having a vinyl group as described in U.S. Patent 2,852,382.

The silver halide or other light-sensitive material used in the photographic element of our invention can be chemically sensitized or optically sensitized by any of the accepted procedures.

Usually our emulsion are coated on photographic supports in the form of multilayer color photographic elements wherein at least three differently sensitized emulsion layers are coated over one another on the support. Usually the support is coated in succession with a red-sensitive layer, a green-sensitive layer, and a blue-sensitive layer either with or without a Carey Lea filter between the blue-sensitive and green-sensitive layers. The three differently color-sensitized layers may be arranged in any other order over one another that is desirable; however, the Carey Lea filter layer obviously would not be put over the blue-sensitive layer. Preferably, these light-sensitive layers are arranged on the same side of the support.

Our invention is further illustrated by the following examples.

#### EXAMPLE 1

The ability of the phenolic coupling agents of our invention to undergo chromogenic development with oxidized developing agent depends on the elimination of the aminoalkyl group located in the coupling position of the coupling agent. The ease of displacement for two of the couplers of our invention was measured by determining the coupling rate relative to phenol. The results are recorded in Table I. The procedure was that of Tong and Glesmann, J.A.C.S., 79, 583 (1957), using a jet-mixing machine described by W. R. Ruby, Rev. Sci. Instruments, 26, 460 (1955).

TABLE I

| Coupler No. | Group in Coupling Position         | Coupling Rate<br>$k \times 10^3$ (relative to<br>phenol = 1 $\times 10^3$ ) |
|-------------|------------------------------------|-----------------------------------------------------------------------------|
| Control     | -H (Guaiacol, control)             | 170                                                                         |
| 1           | -CH <sub>2</sub> NH <sub>2</sub>   | 220                                                                         |
| 6           | -CH <sub>2</sub> NHCH <sub>2</sub> | 240                                                                         |

From the above it can readily be seen that compounds 1 and 6 of our invention are much more reactive than the unsubstituted control, guaiacol.

#### EXAMPLE 2

A single layer gelatin silver bromoiodide emulsion containing coupler 7 and coupler solvent di-n-butylphthalate was made. This coating contained 10 parts of gelatin, 5 parts of silver, 2 parts of coupler, and 1 part of coupler solvent. A strip of the above mentioned coating was given  $\frac{1}{25}$ -second exposure on a 1B intensity scale sensitometer and processed in a conventional manner to a color negative using the following developer solution.

|                                   |       |      |
|-----------------------------------|-------|------|
| Sodium sulfite (anhydrous)        | g     | 2.0  |
| 2-amino-5-diethylaminotoluene HCl | g     | 2.0  |
| Sodium carbonate monohydrate      | g     | 20.0 |
| Potassium bromide                 | g     | 2.0  |
| Water to pH 10.86                 | liter | 1.0  |

The image dye which was formed in the processed strip had a  $\lambda_{max}$  of 690  $\mu\mu$  and a  $D_{max}$  of 2.4.

This processed strip was then immersed in a ferri-

cyanide bleach bath, and the residual coupler formed a yellow dye image (i.e., positive image) which affords automatic color correction by providing a color-correcting mask for the unwanted blue absorption of the cyan dye image. This yellow mask image had a  $\lambda_{\text{max}}$  of 477 m $\mu$  and a  $D_{\text{max}}$  of 0.4.

Similarly, other couplers of our invention are used to advantage in color photography as illustrated previously with representative couplers. Further, the couplers of our invention are valuable as cyan image-forming couplers in multilayer photographic color films containing other classes of couplers in the other layers of said film. Such other couplers are, for example, magenta-forming pyrazolones, cyanoacetyl coumarones, indazolones, etc., and yellow couplers such as  $\alpha$ -acylacetanilides and dibenzoylmethanes.

The preparation of our couplers is illustrated by a description of representative couplers of our invention.

#### COUPLER 1

A solution of 10 g. of vanillin oxime in 200 ml. of ethanol was placed in a bottle of a Burgess-Parr reduction apparatus, 0.2 g. of 10% palladium on carbon catalyst was added, and the mixture shaken at room temperature in an atmosphere of hydrogen under an initial pressure of 50 p.s.i., until the calculated amount was taken up. The catalyst was removed by suction filtration. The filtrate was concentrated to dryness under diminished pressure on a water bath. The crystalline base, melting at 130-132° C., was converted to the hydrochloride and purified by recrystallization from ethanol. The yield of product, melting at 213-214° C., was 8.7 g.

#### COUPLER 2

A mixture of 15.2 g. of vanillin, 7.3 g. of butylamine, and 60 ml. of ethanol was heated at reflux for 30 minutes. The alcohol was distilled under diminished pressure on a water bath. The oily residue, which could not be induced to crystallize, was dissolved in 250 ml. of ethanol and catalytically reduced in the manner described under coupler 1. The hydrochloride, after three recrystallizations from acetonitrile, melted at 128-129° C. The yield of product was 4.6 g.

#### COUPLER 3

A mixture of 18.2 g. of 4-hydroxy-3-methoxybenzylidene aniline, prepared from vanillin and aniline by the benzylidene aniline procedure described in Org. Syn. Coll., vol. I, p. 80, 0.2-0.3 g. of Raney nickel catalyst in absolute ethanol was reduced in a Parr shaker bottle as described under coupler 1. The hydrochloride, obtained by passing dry hydrogen chloride into a benzene solution of the base after two recrystallizations from acetone methanol (1:1 mixture), melted at 162-163° C. The yield of product was 14 g.

#### COUPLER 6

A mixture of 16.7 g. of vanillin oxime, 300 ml. of ethanol, and 0.3-0.5 of Raney nickel catalyst, treated in the manner described under coupler 1 above, gave as the major product, M.P. 245° C. with decomposition.

Couplers 4, 5 and 7 through 23 are prepared by a basic synthesis involving the following steps:

(1) Replacing the hydrogen atom in the 4-position of a 2-substituted phenolic compound with an aldehydic group via a Duff reaction;

(2) Reacting the product of step (1) with an amine to form a Schiff base;

(3) Reducing the Schiff base formed in step (2) to a phenol having an aminomethyl group in the 4-position.

The foregoing procedure may be formulated as follows:



The four-equivalent image-forming couplers of our invention are distinguished from other four-equivalent couplers by having an aminoalkyl group substituted on the coupling position of the coupler molecule. Our couplers are characterized by not producing color fog, and by having very good coupling reactivity. The couplers of our invention may be used in emulsion layers either alone or admixed with other couplers, either four-equivalent couplers, competing couplers, and the like.

The invention has been described in detail with particular reference to preferred embodiments thereof, but it will be understood that variations and modifications can be effected within the spirit and scope of the invention as described hereinabove and as defined in the appended claims.

We claim:

35. An image-forming layer containing silver halide and contiguous thereto a coupler which is capable of forming a cyan dye on coupling with the oxidation product of a primary aromatic amino color developing agent, said coupler containing at least one phenolic coupling moiety, said phenolic coupling moiety being substituted in the coupling position with an aminomethyl group, said amino group having at least one hydrogen atom, and said phenolic coupling moiety being substituted in a position ortho to the hydroxyl group with a group selected from the class consisting of an alkoxy group and an amide group, said dye being nondiffusing.

36. An image-forming layer containing silver halide and contiguous thereto a coupler selected from the class consisting of those having the formulas:



wherein R represents a group selected from the class consisting of an alkoxy group and an amide group; R' represents a group selected from the class consisting of the hydrogen atom, an alkyl group, and an aryl group; R<sup>2</sup> and R<sup>3</sup> each represents a group selected from the class consisting of the hydrogen atom, a halogen atom, an alkyl group, an alkoxy group, an aryl group, and an amide group, and together represent the non-metallic atoms necessary to form a fused ring selected from the class consisting of naphthalene, quinoline, benzothiazole and benzimidazole, said coupler being capable of forming a nondiffusing dye.

37. A light-sensitive hydrophilic colloid silver halide emulsion layer containing 1-hydroxy-4-[N-(4-methoxyphenyl)aminomethyl]-N-[ $\delta$ -(2,4-di-t-amylphenoxy)-butyl]-2-naphthamide.

38. A light-sensitive hydrophilic colloid silver halide

emulsion layer containing 1-hydroxy-4-[N-(4-methoxyphenyl)aminomethyl] - N - octadecyl - N-(3',5'-dicarboxy-2-naphthalenyl)-2-naphthalenylide.

5. A light-sensitive hydrophilic colloid silver halide emulsion layer containing 1 - hydroxy - 4[N - (3-methylphenyl)aminomethyl] - N-octadecyl - 3',5' - dicarboxy-2-naphthalenylide.

6. A light-sensitive hydrophilic colloid silver halide emulsion layer containing 1-hydroxy-4-(N-methylaminomethyl)-2'-tetradecyloxy-2-naphthalenylide.

7. A light-sensitive hydrophilic colloid silver halide emulsion layer containing  $\alpha,\alpha'$ -iminobis{4-methyl-2-[ $\gamma$ -(4-t-butylphenoxy)butyramido]phenol}.

8. An image-forming layer containing silver halide and contiguous thereto a coupler selected from the class consisting of those having the formula:



wherein R represents a group selected from the class consisting of an alkoxy group and an amide group; R' represents a group selected from the class consisting of the hydrogen atom, an alkyl group, and an aryl group; R<sup>2</sup> and R<sup>3</sup> each represents a group selected from the class consisting of the hydrogen atom, a halogen atom, an alkyl group, an alkoxy group, an aryl group, and an amide, and together represent the non-metallic atoms necessary to form a fused ring selected from the class consisting of naphthalene, quinoline, benzothiazole and benzimidazole, said coupler being capable of forming a nondiffusing dye.

9. An image-forming layer of claim 8 in which the R group of the coupler represents an amide group.

10. An image-forming layer containing silver halide and contiguous thereto a coupler selected from the class consisting of those having the formula:



wherein R represents a group selected from the class consisting of an alkoxy group and an amide group; R<sup>2</sup> and R<sup>3</sup> each represents a group selected from the class consisting of the hydrogen atom, a halogen atom, an alkyl group, an alkoxy group, an aryl group, and an amide group, and together represent the non-metallic atoms necessary to form a fused ring selected from the class consisting of naphthalene, quinoline, benzothiazole and benzimidazole, said coupler being capable of forming a nondiffusing dye.

11. A cyan color developer comprising an aqueous alkaline solution containing a primary aromatic amino

70

color developing agent and a diffusible coupler selected from those having the formulas:



wherein R represents a group selected from the class consisting of an alkoxy group and an amide group; R' represents a group selected from the class consisting of the hydrogen atom, an alkyl group, and an aryl group; R<sup>2</sup> and R<sup>3</sup> each represents a group selected from the class consisting of the hydrogen atom, a halogen atom, an alkyl group, an alkoxy group, an aryl group, and an amide group, and together represent the non-metallic atoms necessary to form a fused ring selected from the class consisting of naphthalene, quinoline, benzothiazole and benzimidazole, said coupler reacting with oxidized color developing agent to form a nondiffusing dye.

12. A cyan color developer comprising an aqueous alkaline solution containing a primary aromatic amino color developing agent and a diffusible coupler selected from those having the formulas:



wherein R represents a group selected from the class consisting of a lower alkoxy group and the amide group; R' represents a group selected from the class consisting of the hydrogen atom, a lower alkyl group and phenyl; R<sup>2</sup> and R<sup>3</sup> each represents a group selected from the class consisting of the hydrogen atom, a halogen atom, a lower alkyl group, a lower alkoxy group, phenyl and an amide group and together represent the non-metallic atoms necessary to form a fused ring selected from the class consisting of naphthalene, quinoline, benzothiazole and benzimidazole, said coupler reacting with oxidized color developing agent to form a nondiffusing dye.

13. A cyan color developer comprising an aqueous alkaline solution containing a primary aromatic amino color developing agent and a diffusible coupler selected from the class consisting of 4-aminomethyl-2-methoxyphenol, 4-butylaminomethyl-2-methoxyphenol, 4-anilino-methyl-2-methoxyphenol, 1-hydroxy-4-ethylaminomethyl-2 - naphthamide, 2 - ethoxy - 4-propylaminomethyl-5-acetamido - 1 - naphthol,  $\alpha,\alpha'$  - iminobis(4-methyl-2-methoxyphenol), and 5-(N-ethylaminomethyl)-7-acetamido-8-hydroxyquinoline, said coupler reacting with oxidized color developing agent to form a nondiffusing dye.

60

#### References Cited

#### UNITED STATES PATENTS

- |           |        |                       |        |
|-----------|--------|-----------------------|--------|
| 3,227,550 | 1/1966 | Whitmore et al. ----- | 96—100 |
| 3,227,551 | 1/1966 | Barr et al. -----     | 96—100 |
| 3,311,476 | 3/1967 | Loria -----           | 96—100 |

J. TRAVIS BROWN, Primary Examiner.

U.S. CL. X.R.

96—100; 260—612, 571

UNITED STATES PATENT OFFICE  
CERTIFICATE OF CORRECTIONPatent No. 3,419,390 Dated December 31, 1968Inventor(s) Homer W. J. Cressman and John R. Thirtle

It is certified that error appears in the above-identified patent and that said Letters Patent are hereby corrected as shown below:

Column 9, lines 17 through 27, the structural formula reading



and in line 37, between "amide" and "," insert --group--.  
Column 10, lines 28 through 35, in the structural formula on the right-hand side of the column, that part of the structure readin



SIGNED AND

SEALED

MAY 26 1970

(SEAL)

Attest:

Edward M. Fletcher, Jr.

 Attesting OfficerWILLIAM E. SCHUYLER, JR.  
Commissioner of Patents